

# UNITED STATES PATENT OFFICE.

EDWIN BRYANT THORNHILL, OF GRAY SUMMIT, MISSOURI.

## PROCESS FOR EXTRACTION OF MERCURY FROM ITS ORES AND OTHER MATERIALS.

1,119,377.

Specification of Letters Patent.

Patented Dec. 1, 1914.

No Drawing.

Application filed January 12, 1914. Serial No. 811,592.

To all whom it may concern:

Be it known that I, EDWIN BRYANT THORNHILL, a citizen of the United States of America, and resident of Gray Summit, in the county of Franklin, State of Missouri, in the United States of America, have invented certain new and useful Improvements in Processes for Extraction of Mercury from its Ores and other Materials, of which the following is a specification.

The invention relates to a process for the extraction of mercury from its ores or other materials, and the objects of the invention are to exercise economy in regard to the costs incidental to the production of mercury and to provide an efficient method that will insure a maximum quantity of mercury from a given quantity of the material from which it is extracted, and it consists essentially of the steps in or about the order named, together with the substances used, all being set forth in detail hereinafter and pointed out in the claims for novelty following this description. This method is based on the affinity of mercury sulfid to a solution containing an alkali sulfid and an alkali hydroxid, so that when the ore or other material containing mercury sulfid is treated with this solution, the mercury will leave the original material and go with the solution. The preferable constituents of the solution are sulfid of sodium and hydroxid of sodium.

The solvent, consisting of the solution carrying the mercury that has been extracted, is brought into contact with a metallic substance, aluminum or chromium, or any other metal that is soluble in an alkali hydroxid and does not form the sulfid in the wet way, so that the mercury contained in said solution will be precipitated as finely divided metallic mercury and the metallic substance used as precipitant will go into the solution. The preferable manner of carrying out the withdrawal of the mercury from the solution is to add the metallic precipitant in a finely divided state to the solution during the violent agitation of the latter, thus thoroughly separating all of the mercury from the solution. The mercury withdrawn from the solution in a finely divided state is rubbed or otherwise treated to bring the

small particles into intimate contact with each other and thereby bring said mercury into a fluid condition. The straining of the fluid product through a textile or chamois strainer puts the mercury in a fluid condition for market.

It may be noted that by adding aluminum or chromium to a solution of alkali sulfid, and alkali hydroxid, containing mercury as a sulfid, the sulfur combined with the mercury now combines with the alkali to form an alkali sulfid, the strength of the solution in that chemical is thereby increased.

The reactions are probably as follows:

Dissolving—



Precipitation and regeneration:



What I claim is:

1. The herein described process for the extraction of mercury from its ores and other materials consisting in first treating the ore or other material with an alkali sulfid and an alkali hydroxid in solution and carrying the mercury with said solution, and withdrawing said mercury from said solution by the addition of a precipitant to the latter.

2. The herein described process for the extraction of mercury from its ores and other materials consisting in treating the ore or other material with a solution of alkali sulfid and alkali hydroxid, and adding to the solution a metallic substance as a precipitant, and thereby separating the mercury from said solution.

3. The herein described process for the extraction of mercury from its ores or other materials consisting in treating the ore or other materials with a solution composed of sulfid of sodium and hydroxid of sodium, and thereby carrying the mercury into the solution and adding aluminum to said solution as a precipitant, and thereby separating the mercury from said solution.

4. The herein described process for the extraction of mercury from its ores and other materials consisting in treating the ore or other material with a solution composed of an alkali sulfid and an alkali hydroxid, then

adding a metallic substance to the solution and separating the mercury from the solution, then rubbing the finely divided particles of mercury together, bringing the mercury into a fluid condition, and finally straining the fluid.

Signed at the city of Toronto, this 2d day of December, 1913.

EDWIN BRYANT THORNHILL.

Witnesses:

THOMAS R. JONES,

F. G. HAMMOND.

Copies of this patent may be obtained for five cents each, by addressing the "Commissioner of Patents, Washington, D. C."